

Patented Oct. 12, 1926.

1,602,591

# UNITED STATES PATENT OFFICE.

SAMUEL E. SHEPPARD, OF ROCHESTER, NEW YORK, ASSIGNOR TO EASTMAN KODAK COMPANY, OF ROCHESTER, NEW YORK, A CORPORATION OF NEW YORK.

## PHOTOGRAPHIC LIGHT-SENSITIVE MATERIAL CONTAINING TELLURIUM AND PROCESS OF MAKING THE SAME.

No Drawing. Original application filed June 6, 1924, Serial No. 718,411. Divided and this application filed January 21, 1926. Serial No. 82,846.

This application is a division of my prior application No. 718,411, filed June 6, 1924, for photographic light sensitive materials and processes of making the same, which has 5 matured into Patent 1,574,944, granted Mar. 2, 1926.

This invention relates to the art of photographic materials.

One object of the invention is to provide 10 photographic emulsions, especially developing-out ones, having new or improved properties because of the use or presence therein of materials, the sensitizing properties of which I have discovered. Still another 15 object of my invention is to provide processes in which such materials are used to improve photographic emulsions, especially developing-out ones, as regards light-sensitivity, by which term I include their ability to give the earliest visible impressions or 20 image with the minimum exposure or their ability to give density after a given exposure or both, the usual photographic fluid treatments being used in preparing such impressions or image or density.

A further object of the invention is to provide colloid products, such for instance as gelatins, the usefulness of which for forming light sensitive photographic emulsions, 30 especially developing-out emulsions, is greatly increased and controlled by my said sensitizing materials incorporated therewith. Another object of the invention is to provide processes for preparing said colloid products or intermediates.

Other objects are,—to increase the sensitivity of photographic emulsions, especially developing-out emulsions, while wholly or partially dispensing with expensive or 40 long and uncertain so-called ripening methods; to enable the use of a type of gelatin having desirable physical qualities in making a photographic emulsion of greater light-sensitivity than that normally obtainable with said gelatin; to obtain more stable emulsions through the purity of the ingredients; to increase the light-sensitivity 45 of photographic emulsions, particularly developing-out ones, the grain characteristics of which have already been determined; to increase the general light-sensitivity of such photographic emulsions throughout

the spectral ranges to which they are normally sensitive; to make such photographic emulsions of standard light-sensitive characteristics with gelatins which normally do not produce emulsions having such characteristics; to make, as intermediates in the manufacture of photographic emulsions, gelatins of standard light-sensitivity giving power out of gelatins which do not normally have the power of giving such standard sensitivity to emulsions, such as developing-out ones, made from them. Further objects will hereinafter appear.

I have found that a series of chemical compounds produce remarkable light-sensitizing effects upon photographic emulsions, especially developing-out ones, when incorporated therein. Broadly speaking each 50 compound of these series contains a divalent tellurium atom which is joined by a double bond to a single metalloid atom (not one bond to one atom, and the other bond to a different atom) to which at least another 55 group of atoms is attached. Generally it is desirable that the last mentioned group of atoms be such that it induces in the compound a chemical affinity for silver halids, for instance the compound may combine to 60 an appreciable extent with silver halid to form a soluble complex salt, when said atomic group is present. Moreover, the metalloid atom to which the atom of tellurium is joined by a double bond is in 65 many instances, but not necessarily, a carbon atom.

For some of the preferred examples of my invention, I select from the above series the following subseries tellurocarbamids. As 70 the corresponding carbimids are likewise usable in preferred examples of my invention and are readily changed into said carbamids, especially for instance in emulsions of the alkaline or ammonia type, it will be 75 understood that the corresponding carbimids are included hereinafter when said carbamids are claimed. These subseries of carbamids and carbimids include many compounds containing one or more substituent 80 radicals, such as alkyl, aryl, acyl, alkyl-oxy, aryl-oxy, etc., groups. Examples are allyl 85 isotellurocyanate, allyl tellurourea. Not only can each compound of my series of

light-senstizers be used alone to improve an emulsion (or colloid for an emulsion) but two or more of such compounds may be used together to obtain their mutual or cumulative effects.

It is a common characteristic of the compounds which I use, that said double bonded tellurium atom is chemically held in the molecule with intermediate firmness. 10 Such atom does not react on silver halids as readily as the sulfur atom in sodium sulfide for instance, but it separates out more readily than the sulfur atom in ethyl mercaptan for example. Consequently said 15 double bonded sulfur-group atoms in my compounds correspond roughly in the firmness with which they are held to the firmness with which the sulfur atoms are held in the so-called potential mercaptans, although there is, of course, some range of 20 difference in the firmness with which said double-bonded atoms are held in the different compounds of my series. The sensitiveness of the grains of silver halid in 25 emulsions has been shown to correspond to the presence in said grains of nuclei of unstated chemical composition. I, therefore, attribute the sensitizing action of my 30 compounds to their forming in the emulsion grains small, mostly ultramicroscopic, nuclei which include silver combined with tellurium. The intermediate firmness with which said double-bonded atoms are held in my compounds facilitates this scattered 35 formation or reaction without reacting on the whole of each grain. Since this deduction is not indispensable to the practical using of my invention, I do not wish to be limited to it except as defined in the claims. 40 I have also found that the proportions in which my compounds are incorporated in the emulsions (or in the colloids for the emulsions) are important. If used in too high concentrations, they cause fog, and 45 sometimes reversal. The largest proportions which can be effectively used vary somewhat with the particular sensitizing compound or compounds which are used, with the proportion of gelatin to silver 50 halid in the emulsion, with the type of emulsion as regards grain size characteristics and alkalinity, with the amount of natural sensitizer originating in the gelatin when the latter is manufactured, with the 55 particular silver halid or halids employed, the standard as regards fog which it set by the emulsion maker, etc. This maximum proportion is in any specific case easily found, being about as readily determined 60 by routine test as, for example, the proportion of sulfur permissible in steel for a particular purpose. It is, however, always surprisingly small. In general with gelatino-silver-halid developing-out emulsions, it should be less than about 10 grains

of active sensitizing compound, in 130 pounds of emulsion (the latter being computed as the weight of its non-aqueous ingredients in the dry state); or less than about 10 grains in 100 pounds of gelatin 70 (computed as dry gelatin,) when it is added to the gelatin before the latter is used in making the emulsion. A quantity which causes immediate fogging tendency should not be used,—that is, a quantity 75 which causes more than the tolerated fog allowed in the particular type of emulsion in the trade after the customarily allowed period of storage. I have found 2 to 3 grains of sensitizing compound, to 100 80 pounds of gelatin (computed as dry) or 130 pounds of emulsion (computed as dry) is within the useful limits and generally excellent,—say for instance with alkaline developing-out gelatino-silver-halid emulsions. Of course, smaller amounts of sensitizers are employed when less sensitizing effects are desired; but it is important not to exceed the upper limits as stated above. 85

Because only very minute quantities of 90 my sensitizing compounds are used, (often less than one three hundred thousandth of the weight of the emulsion) the addition of them does not appreciably dilute the emulsion or emulsion-forming colloid; nor 95 does it affect their physical properties. Consequently the use of my compounds provides a novel, dependable, and independent way for controlling the properties 100 of photographic emulsions in addition to the customary expedients hitherto available. Gelatins, for instance, can be selected for their physical properties, such as setting ability, melting point and viscosity, without regard to whether they can be made 105 into sufficiently light-sensitive emulsions, and any deficiency in sensitizing power can be made up by incorporating a little quantity of one or more of my independent compounds. Nor are the grain-size characteristics affected by such additions of my compounds, they being independently controlled 110 by the emulsion maker. In other words, I can establish a ratio of sensitizing compounds to silver halid in the emulsions 115 which is independent of the ratio of gelatin to silver halid. Still differently stated, the sensitizer compounds can be added without adding any colloid, such as gelatin, and are, therefore, independent thereof. 120

My sensitizing compounds act as so-called "chemical" sensitizers instead of as "optical" sensitizers. In other words, they increase the "general" sensitiveness of photographic emulsions, notably developing-out ones, in which they are incorporated,—that is to light of substantially the same wave lengths as those to which the emulsion would be sensitive without the incorporation of my compounds; instead of merely increasing the 125 130

sensitiveness to some narrow group of wave lengths. Unlike the effects of dyes, the sensitiveness is increased throughout the normal spectral range of the emulsion instead of at only those spectral points corresponding to the spectral absorption of the sensitizing compound. My compounds are effective in increasing the general light-sensitiveness of orthochromatic, panchromatic, X-ray, and all special emulsions, as well as the ordinary or non-color sensitized ones. They can be added without or with sensitizing dyes or before or after them. They do not specifically affect the dye action; but simply increase the general sensitiveness and thus increase the ordinary sensitiveness to blue light to at least as great an extent as to light of a color corresponding to the dye.

My sensitizing compounds may be used in many ways. Broadly they may be incorporated in emulsions or in colloids for emulsions or both. They can also enter the emulsion mixed with other ingredients thereof whether organic or inorganic. They may be added at different stages of emulsion manufacture, even when the latter is otherwise completely ready for coating. Since their action is rapid when incorporated, the coating in such case need be delayed only long enough to mix in the sensitizing compounds. With the grain characteristics, such as size distribution, etc., already determined, and the other physical and photographic properties of the emulsion already taken care of at this stage, I can practically independently increase its light-sensitiveness without impairing said other properties by adding one or more of my compounds. The latter are especially effective in emulsions which are, at least slightly, alkaline.

Where different batches of emulsion, especially developing-out emulsions, fall below a required manufacturing standard of light sensitiveness, although they may be otherwise satisfactory, their sensitiveness can readily be brought up to standard by mixing in my sensitizing compounds, the proportion varying with the increase necessary to produce a uniform product. Emulsions having almost no practical light-sensitiveness but having enough other desirable qualities can be made usefully light-sensitive by my compounds. Thus the latter are useful in connection with emulsions having good initial light-sensitiveness and those having almost no initial sensitiveness. The increase in sensitiveness can be effected in one step by thoroughly stirring all of the sensitizing compound into the emulsion at one time; or it may be incorporated part at a time in successive steps. When making new batches of emulsion from the same materials which have yielded deficient emulsions, correctional quantities of my sensitizing compounds can

be premixed with an ingredient, such as gelatin.

The following example illustrates how light-sensitive photographic emulsions of the developing-out type may be prepared and improved by the aid of one or more of my sensitizing compounds. Of course, my invention is not restricted to this illustration, except as indicated in the claims. The emulsion-forming operations hereinafter described are along the lines of known practice, see for instance "Die Photographie mit Bromsilber Gelatin" by J. M. Eder, published in Halle, Germany in 1903 by Wilhelm Knapp as part III of Eder's "Ausführliches Handbuch der Photographie."

The two following solutions are made up, the parts being by weight:

A. 900 parts of silver nitrate in 9,200 parts of water.

B. 690 parts of potassium bromide and 50 parts of potassium iodide in 6,100 parts of water along with 300 parts of gelatin.

In mixing B, the halid salts are first dissolved, the water and the gelatin then added to the salt solution. Solution B is then warmed, say to 140° F. or 150° F. for example and the silver nitrate solution A is gradually added to it with constant stirring. It is preferable to warm solution A before adding it to B, say to 150° F. or 160° F. for instance. When solution A has been thoroughly incorporated in solution B, there are then added 43 parts of strong ammonia previously dissolved in 900 parts of water. The emulsion formed by these operations is allowed to stand for a short time, say 15 minutes to a half hour for example. Then 1050 parts of gelatin are dissolved in it with thorough mixing. The emulsion is next cooled, such as by keeping in a cool space, until it sets to a firm jelly. The latter is broken up, as by shredding for instance, and thoroughly washed to remove soluble salts, such as potassium nitrate and any excess potassium halids. The wash water is, of course, cool enough not to melt the pieces of emulsion jelly. The washed emulsion is next remelted to 100° F. and 1050 parts of water soaked gelatin are thoroughly mixed into it, the temperature then being raised, say between 120° F. and 150° F., for instance, for a short time, say a few minutes. It is then cooled and set. It is an example of the ammonia or alkaline type of developing-out emulsion.

My sensitizing compounds may be usefully incorporated at any stage of the above described process of preparing the emulsion, even being premixed with solutions A or B or with ammonia or with the gelatin, at the initial stages. When the compounds are incorporated in either a partly or wholly prepared emulsion, they are most conveniently handled by dissolving them in a solvent which is inert with respect to the emulsion

and simply acts as a vehicle to help in spreading the compounds throughout the emulsion. So long as an even distribution of the compounds throughout the emulsion is effected and the correct proportion of them is added, their particular concentration in the solvent or vehicle is not important. It is good practice to keep the volume of the solution added to the emulsion under 2% of the volume of the emulsion; but this is not indispensable. For example, where 1 part of allyl tellurourea by weight is to be incorporated into 300,000 parts by weight of the above described emulsion (computed as the weight of its non-aqueous ingredients) the emulsion is melted, the sensitizer dissolved in ethyl alcohol or water or a mixture of them, the volume of said solvent being under approximately 1.5% of the volume of the melted emulsion, and then the solution is thoroughly mixed into the emulsion. When necessary to minimize dilution, the volume of solution can be kept even below a fraction of 1%. I may mention also as very useful potassium tellurocyanide.

With its light-sensitiveness increased by my compounds, the emulsion, being melted to the desired flowability, is coated on its support such as glass, film, paper, etc., in the well known way. It is convenient to control and check the process by coating samples of the emulsion before and after the addition of my sensitizing compounds, the coated specimens being tried out photographically by any well known sensitometric test, or even by comparative camera exposure on the same subject under like conditions. Of course, the usual precautions are observed during the emulsion making and coating processes, such as the use of non-actinic or "safe" light, cleanliness of vessels and air, etc.

The different gelatines sold for photographic emulsion-making may be used in the example given above, hard ones being very useful. The temperatures given are, of course, adjusted if the particular gelatin employed has physical properties, such as melting and setting points, which deviate considerably from the usual ones, such adjustment being a matter of routine control.

Instead, however, of using gelatins which give emulsions of useful but lower sensitiveness even before the addition of my sensitizing material, an almost inert gelatin may be employed,—one which forms an emulsion which produces a developable image, if at all, only after impractically long exposures, and then does not yield an image of desirable density. A gelatin which forms such a practically inert emulsion may be prepared in the way described under the heading "Preparation of ash-free gelatin" in pages 1856 and 1859 of the "Journal of the American Chemical Society", September, 1922, vol. XLIV, No. 9, being part of an article

by Sheppard, Sweet, and Benedict on "Elasticity of purified gelatin jellies as a function of hydrogen-ion concentration." Emulsions of impractically low light-sensitiveness made by the above described process from such prepared gelatin, are transformed by my sensitizing compounds into emulsions which give developable images of excellent density after usefully brief exposures. I have, for example, been able to increase the light-sensitiveness of some such low sensitive emulsions ten or even over twenty times, the exposures for a given subject in the latter case being cut to less than one twentieth of the original one and the image density being made excellent by a corresponding gain. Increases of the same general order of magnitude are made when my sensitizing compounds are added in similar proportions to emulsions which are made from normal photographic gelatins or mixtures of such normal gelatins with said almost inert gelatins, and already have useful, but lower initial sensitiveness. Different percentages of sensitizer produce correspondingly different increases. The increases in developing-out emulsions appear upon the usual developing operations. Customary pyro and metol-hydrochinon alkaline developers are suitable for example. An inert emulsion prepared as above described is a very useful medium or standard in which to test the sensitizing properties of different compounds, a sample containing the compound under test being tried out photographically along with a parallel sample of unsensitized emulsion.

Instead of the inert gelatin prepared according to the reference given in the preceding paragraph, I can prepare inert gelatins by treating active photographic gelatins with oxidizing agents. The latter oxidize the sulfur in the sensitizing substituted (allyl) thiocarbamide or corresponding carbimide, which occurs naturally in photographic gelatins, thus converting it to a non-sensitizing compound and leaving the gelatins practically inert. Dilute aqueous solutions of a peroxide, such as sodium peroxide (say from 5 to 10% by weight) is intimately mixed into the gelatin and then washed out when the oxidation has occurred. The inert gelatin referred to in the preceding paragraph can be thus oxidized to make its inertness doubly sure.

When preparing inert gelatin on a considerable scale, it is far preferable to introduce the oxidizing step during the regular manufacturing operations, say the liming and/or deliming treatments. The oxidizing agents should be effective as desensitizers and yet not be present in quantities capable of materially reducing the yield of gelatin or harming its quality, especially its physical properties. Nor should they leave objectionable products from the oxidation re-

action. For example, the regular liming solution of the usual gelatin manufacturing process can be saturated with as much calcium hypochlorite as will dissolve therein; 5 or it can obtain about 5 to 10% of sodium peroxide. Subsequent operations then proceed as usual.

My sensitizing compounds may be incorporated into gelatin from which photographic 10 emulsions are to be made. This "strengthened" gelatin then constitutes a valuable "intermediate" in emulsion manufacture. While any good gelatin may be thus treated, that which has been rendered inert by the 15 above described oxidation treatment during liming or deliming is particularly adapted to this strengthening. Emulsions made from the mixture have markedly increased light-sensitivity as compared with those made 20 from corresponding unstrengthened gelatins. The proportion of sensitizing material is, of course, adjusted to give the desired control of the sensitivity of emulsions made from the gelatin, the total sensitizing material in 25 the "strengthened" gelatin being thus brought to, or even above, normal.

When working on a considerable scale, this activating of gelatin, such, for instance, as said inert gelatin, is one of the most desirable ways of employing my sensitizing 30 compounds. In fact, premixing of one or more of my sensitizers with gelatin is my preferred system. During manufacture of the gelatin, say for instance when the concentrated gelatin solution comes from the evaporator before setting and drying, the sensitizing compound or compounds are added and thoroughly mixed to obtain effectively uniform distribution. For example 2 35 or 3 grains of any of the hereinabove listed compounds or mixtures of them is carefully mixed with each fraction of gelatin solution containing 100 pounds of gelatin (calculated as dry). The compound is taken up, 40 preferably in as little aqueous-alcohol mixture as is practicable, and then this concentrated solution added to the gelatin solution. In this way undesirable dilution 45 of the latter is avoided.

On a large scale, the sensitized solution 50 may be accurately and continually dosed into a regulated stream of gelatin solution with continuous mixing. Alternately dried or set gelatin may be allowed to swell in an 55 aqueous solution of the sensitizing compound. The nearly uniform distribution or diffusion of the compound in the gelatin thus effected can be made even more nearly uniform by melting and agitating the swollen gelatin.

In the examples given above, the steps of treating with ammonia and warming of the emulsion just before its final setting improve the photographic properties of the emulsion, especially when the latter is made

from hard gelatins. But one or both of them may be omitted. In other words, my sensitizing compounds act by themselves to increase the light-sensitivity, whether ripening steps be employed or not, and so 70 can wholly or partially replace them. But I prefer to use them because the effect of either or both of them is to help increase the light-sensitivity of the emulsions and thus gives a stronger initial sensitized condition which is multiplied or increased by 75 using my sensitizing compounds. When using any of the inert gelatins mentioned above in making very sensitive emulsions, these steps can sometimes be shortened and 80 made more certain in effect by reason of the use of my powerful and dependable sensitizing compounds.

I have described gelatin emulsions and emphasized the developing-out and alkaline 85 types because at the present time they are the ones which have the widest practical use. Moreover they form the best medium for testing new sensitizing-compounds. But other organic colloids and mixtures of them 90 with each other or with gelatin, where their nature admits such mixtures, may be used in making light-sensitive emulsions which can be improved by adding my sensitizing material. Albumens, agar-agar, gums, such 95 as gum-arabic, cellulosic derivatives such as collodion are instances. While I have illustrated the use of my sensitizer in connection with such sensitive substances as silver bromide and silver iodide, other light- 100 sensitive substances can be employed, such as silver chlorid, alone or mixed with one or more of the others.

Having thus described my invention, what I claim as new and desire to secure by 105 Letters Patent is:

1. A photographic developing-out emulsion comprising a colloid, particles of photographic silver salt suspended therein, and an added compound therein upon which 110 at least part of the light-sensitivity of the emulsion depends, said compound containing a divalent tellurium atom directly joined by a double bond to a single metalloid atom to which at least another group of 115 atoms is attached, the proportion of said compound being substantially independent of the proportion of said colloid.

2. A photographic developing-out emulsion comprising gelatin, particles of silver 120 halid suspended therein and telluro carbamid upon which at least part of the light-sensitivity of the emulsion depends.

3. A photographic developing-out emulsion comprising gelatin, particles of silver 125 halid suspended therein and allyl tellurourea upon which at least part of the light-sensitivity of the emulsion depends.

4. A photographic developing-out gelatino-silver-halid emulsion of the alkaline

type of relatively high light-sensitiveness, comprising a mixture of the constituents of a gelatino-silver-halid emulsion of lower light-sensitiveness and an added sensitizing compound upon which depends the difference between said lower and said high light sensitiveness, said compound containing a divalent tellurium atom directly joined by a double bond to a single metalloid atom to which at least another group of atoms is attached.

5 5. A photographic emulsion comprising a colloid, particles of silver halid suspended therein and an added compound therein upon which at least part of the light-sensitiveness of the emulsion depends, said compound containing a divalent tellurium atom directly joined by a double bond to a single metalloid atom to which at least another 10 group of atoms is attached, the proportion of said compound being substantially independent of the proportion of gelatin, and said emulsion being substantially free from sensitizing dye.

15 6. A photographic developing-out emulsion comprising a colloid, particles of photographic silver salt suspended therein, and an added compound therein upon which at least part of the light-sensitiveness 20 of the emulsion depends, said compound containing a divalent tellurium atom directly joined by a double bond to a single metalloid atom to which at least another group of atoms is attached, the amount of 25 added compound being less than the order of 10 grains per 130 pounds of emulsion and insufficient to cause immediate fogging tendency.

30 7. In a process of preparing a developing-out gelatino-silver-halid emulsion, increasing the light-sensitiveness thereof by incorporating with the other constituents thereof a sensitizing compound containing a divalent tellurium atom directly joined by 35 a double bond to a single metalloid atom to which at least another group of atoms is attached.

40 8. In the process of preparing a developing-out gelatino-silver-halid emulsion, increasing the light-sensitiveness thereof by incorporating a telluro carbamid with the other constituents thereof.

45 9. In the process of preparing a developing-out gelatino-silver-halid emulsion, increasing the light-sensitiveness thereof by incorporating allyl tellurourea with the other constituents thereof.

50 10. In the process of preparing a developing-out gelatino-silver-halid emulsion of the alkaline type of relatively high light-sensitiveness, combining constituents of a gelatino-silver-halid emulsion of said type but of lower light-sensitiveness with an independent sensitizing compound, said compound containing a divalent tellurium atom

of the sulfur group directly joined by a double bond to a single metalloid atom to which at least another group of atoms is attached.

11. In the process of preparing a developing-out colloid sensitive-silver-salt emulsion, increasing the light-sensitiveness thereof by incorporating with the other constituents thereof, which are substantially free from sensitizing dye, a sensitizing compound, which is also substantially free from sensitizing dye, said compound containing a divalent tellurium atom directly joined by a double bond to a single metalloid atom to which at least another group of atoms is attached.

12. In the process of preparing a developing-out gelatino-silver-halid emulsion, increasing the light-sensitiveness thereof by incorporating with the other constituents thereof a sensitizing compound containing a divalent tellurium atom directly joined by a double bond to a single metalloid atom to which at least another group of atoms is attached, the amount of said added compounds being less than the order of 10 grains per 130 pounds of emulsion and insufficient to cause immediate fogging tendency.

13. An intermediate for use in making photographic emulsions, comprising an emulsion-forming colloid having incorporated therein a sensitizing compound containing a divalent tellurium atom directly joined by a double bond to a single metalloid atom to which at least another group of atoms is attached.

14. An intermediate for use in making photographic emulsions, comprising gelatin having incorporated therein telluro carbamid.

15. An intermediate for use in making photographic emulsions, comprising gelatin having incorporated therein allyl tellurourea.

16. An intermediate for use in making photographic emulsions, comprising an emulsion-forming colloid having incorporated therein a sensitizing compound containing a divalent tellurium atom directly joined by a double bond to a single metalloid atom to which at least another group of atoms is attached, the amount of said added compound being less than the order of 10 grains in 100 pounds of gelatin.

17. The process of making an intermediate for use in the preparation of photographic emulsions, which comprises incorporating in an emulsion-forming colloid an independent sensitizing compound containing a divalent tellurium atom directly joined by a double bond to a single metalloid atom to which at least another group of atoms is attached.

18. The process of making an intermediate for use in the preparation of photo-

- graphic emulsions, which comprises incorporating in an emulsion-forming colloid telluro carbamid.
19. The process of making an intermediate for use in the preparation of photographic emulsions, which comprises incorporating in an emulsion-forming colloid allyl tellurourea.
20. The process of making an intermediate for use in the preparation of photographic emulsions, which comprises incorporating in an emulsion-forming colloid an independent sensitizing compound containing a divalent tellurium atom directly joined by a double bond to a single metalloid atom to which at least another group of atoms is attached, the amount of said added compound being less than the order of 10 grains per 100 pounds of said colloid (calculated as dry colloid), and being insufficient to cause immediate fogging tendency.
21. The process of making an intermediate for use in the preparation of photographic emulsions, which comprises incorporating in an emulsion-forming colloid telluro carbamid, the amount of said added compound being less than the order of 10 grains per 100 pounds of said colloid (calculated as dry as colloid) and being insufficient to cause immediate fogging tendency.
22. The process of making an intermediate for use in the preparation of photographic emulsions, which comprises incorporating in an emulsion-forming colloid allyl tellurourea, the amount of said added compound being less than the order of 10 grains per 100 pounds of said colloid (calculated as dry colloid) and being insufficient to cause immediate fogging tendency.
23. The process of making an intermediate for use in the preparation of photographic gelatino-silver-halid emulsions, which comprises substantially freeing gelatin from sensitizing compounds, and incorporating therein a sensitizing compound containing a divalent tellurium atom directly joined by a double bond to a single metalloid atom to which at least another group of atoms is attached.
24. The process of making an intermediate for use in the preparation of photographic gelatino-silver-halid emulsions, which comprises substantially freezing gelatin from sensitizing compounds, and incorporating therein telluro carbamid.
25. The process of making an intermediate for use in the preparation of photographic gelatino-silver-halid emulsions, which comprises substantially freeing gelatin from sensitizing compounds, and incorporating therein a sensitizing compound containing a divalent tellurium atom directly joined by a double bond to a single metalloid atom to which at least another group of atoms is attached, the amount of said added compound being less than the order of 10 grains for 100 pounds of gelatin (calculated as dry gelatin), and being insufficient to cause immediate fogging tendency in emulsions made from said intermediate.

Signed at Rochester, New York, this 18th day of January, 1926.

SAMUEL E. SHEPPARD.

graphic emulsions, which comprises incorporating in an emulsion-forming colloid telluro carbamid.

19. The process of making an intermediate for use in the preparation of photographic emulsions, which comprises incorporating in an emulsion-forming colloid allyl tellurourea.

20. The process of making an intermediate for use in the preparation of photographic emulsions, which comprises incorporating in an emulsion-forming colloid an independent sensitizing compound containing a divalent tellurium atom directly joined by a double bond to a single metalloid atom to which at least another group of atoms is attached, the amount of said added compound being less than the order of 10 grains per 100 pounds of said colloid (calculated as dry colloid), and being insufficient to cause immediate fogging tendency.

21. The process of making an intermediate for use in the preparation of photographic emulsions, which comprises incorporating in an emulsion-forming colloid telluro carbamid, the amount of said added compound being less than the order of 10 grains per 100 pounds of said colloid (calculated as dry as colloid) and being insufficient to cause immediate fogging tendency.

22. The process of making an intermediate for use in the preparation of photographic emulsions, which comprises incorporating in an emulsion-forming colloid allyl tellurourea, the amount of said added compound being less than the order of 10 grains per 100 pounds of said colloid (cal-

culated as dry colloid) and being insufficient to cause immediate fogging tendency.

23. The process of making an intermediate for use in the preparation of photographic gelatino-silver-halid emulsions, which comprises substantially freeing gelatin from sensitizing compounds, and incorporating therein a sensitizing compound containing a divalent tellurium atom directly joined by a double bond to a single metalloid atom to which at least another group of atoms is attached.

24. The process of making an intermediate for use in the preparation of photographic gelatino-silver-halid emulsions, which comprises substantially freezing gelatin from sensitizing compounds, and incorporating therein telluro carbamid.

25. The process of making an intermediate for use in the preparation of photographic gelatino-silver-halid emulsions, which comprises substantially freeing gelatin from sensitizing compounds, and incorporating therein a sensitizing compound containing a divalent tellurium atom directly joined by a double bond to a single metalloid atom to which at least another group of atoms is attached, the amount of said added compound being less than the order of 10 grains for 100 pounds of gelatin (calculated as dry gelatin), and being insufficient to cause immediate fogging tendency in emulsions made from said intermediate.

Signed at Rochester, New York, this 18th day of January, 1926.

SAMUEL E. SHEPPARD.

#### Certificate of Correction.

It is hereby certified that in Letters Patent No. 1,602,591, granted October 12, 1926, upon the application of Samuel E. Sheppard, of Rochester, New York, for an improvement in "Photographic Light-Sensitive Material Containing Tellurium and Processes of Making the Same," errors appear in the printed specification requiring correction as follows: Page 1, line 43, after the word "making" insert the word *such*; page 2, line 56, after the word "which" insert the word *is*; page 3, line 22, for the article "The," first occurrence, read *They*; page 5, line 50, for the word "sensitized" read *sensitizing*; same page, line 53, for the word "Alternately" read *Alternatively*; page 6, line 39, claim 7, for the article "a," first occurrence, read *the*; page 7, line 29, claim 21, strike out the word "as"; same page, line 53, claim 24, for the word "freezing" read *freeing*; and that the said Letters Patent should be read with these corrections therein that the same may conform to the record of the case in the Patent Office.

Signed and sealed this 28th day of December, A. D. 1926.

[SEAL.]

M. J. MOORE,  
Acting Commissioner of Patents.

**Certificate of Correction.**

It is hereby certified that in Letters Patent No. 1,602,591, granted October 12, 1926, upon the application of Samuel E. Sheppard, of Rochester, New York, for an improvement in "Photographic Light-Sensitive Material Containing Tellurium and Processes of Making the Same," errors appear in the printed specification and requiring correction as follows: Page 1, line 43, after the word "making" insert the word *such*; page 2, line 56, after the word "which" insert the word *is*; page 3, line 22, for the article "The," first occurrence, read *They*; page 5, line 50, for the word "sensitized" read *sensitizing*; same page, line 53, for the word "Alternately" read *Alternatively*; page 6, line 39, claim 7, for the article "a," first occurrence, read *the*; page 7, line 29, claim 21, strike out the word "as"; same page, line 53, claim 24, for the word "freezing" read *freeing*; and that the said Letters Patent should be read with these corrections therein that the same may conform to the record of the case in the Patent Office.

Signed and sealed this 28th day of December, A. D. 1926.

[**SEAL.**]

**M. J. MOORE,**  
*Acting Commissioner of Patents.*